

## UNITED STATES PATENT OFFICE

2,336,265

## COATED FABRIC

Robert L. Lester, Newburgh, N. Y., assignor to E. I.  
du Pont de Nemours & Company, Wilmington,  
Del., a corporation of Delaware

No Drawing. Application August 20, 1941,  
Serial No. 407,608

3 Claims. (Cl. 117—166)

This invention relates to the production of coated fabrics, and more particularly to the production of shade cloth for window shades and the like, having improved properties.

Window shade cloth comprising a textile fabric coated with a cellulose nitrate composition is well known in the art of coated fabrics and has been developed to a point where it is considered generally satisfactory. However, there is need for improvement where the shade cloth is subjected to sunlight exposure over a long period of time. A serious objection of the present-day material is technically referred to as tendering. By "tendering" is meant that a shade cloth loses after prolonged exposure to sunlight much of its original tensile strength. A further objection of the prior art material is a lack of color stability, particularly in the case of white and other light colored translucent shade cloth materials.

It is well known that zinc oxide is an excellent filter for ultra violet light and, for this reason, it has been used quite extensively in pyroxylin coatings for window shade material to filter ultra violet light which is known to have a deleterious effect on nitrocellulose. By the use of zinc oxide in pyroxylin coatings for window shade material definite improvements have been made with respect to tendering. However, there is need for further improvement since the grades of zinc oxide normally used do not give completely satisfactory results with respect to tendering and color stability.

An object of the present invention is the provision of an improved shade cloth material. A further object is to provide a shade cloth material having great resistance to tendering when exposed to sunlight over a prolonged period. A further object is to provide a shade cloth material having great resistance to color change, particularly in the case of white and other light colored shade cloth material, when exposed to sunlight over a prolonged period.

The objects of this invention are accomplished by coating each side of a textile fabric base material with a liquid coating composition comprising a solution of nitrocellulose, a plasticizer, and pigment. At least 20% of the total pigment in the coating composition consists of zinc oxide particles, the size of which is greater than .4 micron in any one direction.

During recent years in the pigmented coating art the tendency has been toward smaller and smaller pigment particles with the aim of increasing the covering power and increasing the gloss of the coating. The particle size of pig-

ments have been reduced to less than the wavelength of ultra violet light which is less than 4,000 angstroms which corresponds to .4 micron. In a systematic study of the effect of the particle size of zinc oxide pigments upon the tensile strength and color stability of window shade material coated with a composition containing such pigments, it was found that particles having a greater diameter than .4 micron or in the case of acicular shaped particles, those having a width greater than .4 micron, deteriorated less than similar material containing zinc oxide particles less than .4 micron under simultaneous conditions of exposure. It was also discovered that there was greater color stability in the case of the material employing the larger particles of zinc oxide.

An accelerated test for window shade material is obtained by exposing the material at Hialeah, Florida, in a closed box with a glass cover for a period of 40 weeks. The material is positioned in the box four inches from the glass at an angle of 45° and facing south. The surface temperature of the window shade material when exposed under these conditions often reaches 200° F. due to lack of circulation of air inside the exposure box. This temperature is far in excess of any temperature the window shade material is exposed to in actual service. The exposure in Florida as described corresponds to approximately 10 years of service under normal conditions.

The following examples are given to illustrate specific embodiments of the invention, although it is to be understood that the invention is in no way limited to these particular examples.

To a suitable sheeting, such as one running 4.95 yards per pound at a width of 37½ inches, and having a thread count of 68 x 72, is applied by means of a doctor knife on each side a total of 0.3 to 0.8 ounce, dry weight, per square yard, which corresponds to a total of 0.6 to 1.6 ounces per square yard on both sides of a suitable liquid coating composition. After the volatile solvents of the coating composition are expelled by passing the material through a heated chamber, the coated fabric is then subjected to a pressure treatment by passing the material between heated pressure rolls. The rolls may be either smooth or have shallow engraving upon them, such as a Skiver design or the like. The material is finished by applying an additional amount of a suitable coating composition to each side of the fabric. The amount of coating composition applied after pressure treatment is the same as that applied before pressure treatment, viz., 0.3 to 0.8

ounce on each side, dry weight per square yard. The total amount of dry coating on both sides of the fabric corresponds to 1.2 to 3.2 ounces per square yard.

In the case of translucent window shade material the dry coating composition may be as follows:

|                   | Parts by weight |
|-------------------|-----------------|
| Cellulose nitrate | 53.8-40.6       |
| Pigment           | 18.0-28.0       |
| Dibutyl phthalate | 28.2-31.4       |

| Particular size of zinc oxide particles in coating | Initial tensile strength |    |           | Tensile strength after 20 weeks' Florida exposure |    |           |                        | Tensile strength after 40 weeks' Florida exposure |    |           |                        |
|----------------------------------------------------|--------------------------|----|-----------|---------------------------------------------------|----|-----------|------------------------|---------------------------------------------------|----|-----------|------------------------|
|                                                    | W.                       | F. | W. and F. | W.                                                | F. | W. and F. | Per cent deterioration | W.                                                | F. | W. and F. | Per cent deterioration |
| Nodular (diameter): .25 to .30 micron              | 68                       | 46 | 114       | 57                                                | 35 | 92        | 19                     | 48                                                | 19 | 67        | 41                     |
| Aciular—                                           |                          |    |           |                                                   |    |           |                        |                                                   |    |           |                        |
| Width .54 micron, length 3.2 microns               | 73                       | 46 | 119       | 72                                                | 46 | 118       | 1                      | 63                                                | 37 | 100       | 16                     |
| Width .43 micron, length 3.2 microns               | 69                       | 46 | 115       | 67                                                | 41 | 108       | 6                      | 62                                                | 36 | 98        | 15                     |
| Width .43 micron, length 3.2 microns               | 67                       | 42 | 109       | 62                                                | 40 | 102       | 6                      | 63                                                | 36 | 99        | 9                      |

In the case of the so-called opaque material the dry coating composition may be as follows:

|                   | Parts by weight |
|-------------------|-----------------|
| Cellulose nitrate | 43.0-25.0       |
| Pigment           | 45.0-56.3       |
| Dibutyl phthalate | 12.0-18.7       |

The method of preparing the above compositions which comprises dissolving the cellulose nitrate in organic solvents to form a solution and grinding the pigment in the plasticizer before blending with the solution is well known in the art and forms no part of the present invention and a detailed description of such method does not appear to be necessary.

Duplicate samples of white translucent window shade material were made employing nodular shaped zinc oxide as the total pigment content. In one case the diameter of the zinc oxide pigment particles corresponded to 1.0 to 1.5 microns and in the other case the diameter of the zinc oxide pigment particles corresponded to .25 to .30 micron. Both materials were exposed simultaneously at Hialeah, Florida, under glass and four inches from the glass facing south at an angle of 45° for a period of 40 weeks. The tensile strength of each material was measured before exposure, at the end of 20 weeks' exposure, and at the end of 40 weeks' exposure.

The following table indicates the results of deterioration of tensile strength of window shade material employing nodular shaped zinc oxide as the total pigment content:

| Diameter of nodular zinc oxide particles in coating | Initial tensile strength |    |           | Tensile strength after 20 weeks' Florida exposure |    |           |                       | Tensile strength after 40 weeks' Florida exposure |    |           |                       |
|-----------------------------------------------------|--------------------------|----|-----------|---------------------------------------------------|----|-----------|-----------------------|---------------------------------------------------|----|-----------|-----------------------|
|                                                     | W.                       | F. | W. and F. | W.                                                | F. | W. and F. | Percent deterioration | W.                                                | F. | W. and F. | Percent deterioration |
| .25 to .30 micron                                   | 61                       | 49 | 110       | 52                                                | 32 | 84        | 24                    | 39                                                | 19 | 58        | 47                    |
| 1.0 to 1.5 microns                                  | 70                       | 49 | 119       | 67                                                | 41 | 108       | 9                     | 56                                                | 32 | 88        | 26                    |

The white material containing the smaller zinc oxide pigment particles had definitely yellowed at the end of the 40 weeks' exposure and the similar material containing the larger particles did not develop any substantial yellowing during the same period.

Material which deteriorates more than 35% in tensile strength upon 40 weeks of Florida exposure is considered unsatisfactory for com-

mercial use and material which deteriorates less than 35% upon 40 weeks of Florida exposure is considered satisfactory for commercial use and is acceptable to the trade in general.

5 The following table indicates the results obtained with acicular shaped zinc oxide pigment particles incorporated in the coating composition. Inasmuch as acicular zinc oxide particles are not available in widths less than .4 micron, the 10 nodular shaped zinc oxide having a diameter of .25 to .30 micron was employed as a control for the following tests:

25 At the end of the 40 weeks' exposure in Florida, the original tensile strength of the window shade material containing the nodular shaped particles ranging in diameter from .25 to .30 micron had deteriorated 41%; whereas the original tensile 30 strength of the material containing the larger acicular shaped particles only deteriorated 9% to 16%. The material containing the smaller particles of zinc oxide developed a yellow cast during the exposure period; whereas the material 35 containing the larger particles did not undergo any color change.

These results are surprising since in the paint and lacquer field the tendency is to increase the hiding power by decreasing the size of the pigment particles. Therefore, one skilled in the art 40 who was confronted with the problem of producing a shade cloth material capable of filtering ultra violet light to prevent tendering would undoubtedly resort to the smaller pigment particles to accomplish increased hiding power.

It is probable that the yellow color which develops in the case of material containing the smaller particles of zinc oxide results from the 50 decomposition of the nitrocellulose binder rather than any color change of the pigment.

In order to make a wide range of colors in window shade material it is necessary to blend the zinc oxide pigments with various colored pigments, such as carbon black, bone black, chrome green, chrome yellow, ultramarine blue, iron oxide and various colored lakes.

The advantages of this invention do not accrue if the large particle size zinc oxide (greater than .4 micron in all dimensions) is present in 70 amounts less than 20% of the total pigment content of the dry coating composition. The advantages of this invention are accomplished by employing large particle size zinc oxide which may vary between 20% to 100% of the total dry pigment content.

The compositions given in the examples are merely illustrative. Any well known softener may be used in the composition such as castor oil, blown cottonseed oil, blown rapeseed oil, or the like, but it is preferred to employ a so-called "solvent softener," such as dibutyl phthalate, dibutyl tartrate, etc., and resinous plasticizer since the solvent softeners tend to reduce the tendency of the shade cloth to curl as is disclosed in U. S. Patent 2,033,170.

To obtain the improved results of the present invention, it has been found that zinc oxide, either the pure or leaded varieties, must be employed. The zinc oxide pigment may be either of acicular or nodular shape. In the case of acicular shaped particles of zinc oxide, the smallest dimension (width) of the particle should not be less than .4 micron.

The proportions given in the example are merely illustrative and may be varied over a wide range as will be readily apparent to those skilled in the art, the proportions being governed by the desired degree of translucency. In the case of equal weights of coating on the window shade material, the greater the amount of pigment the less is the amount of light transmitted and vice versa.

In the example the fabric employed was a woven cotton sheeting and is the usual type of fabric employed for window shade material although other types of fabric may be employed.

The outstanding advantage of shade cloth produced in accordance with the present invention is the resistance of the material to tendering upon prolonged exposure to sunlight and heat, and a much greater life than window shade material produced in accordance with the prior art. A further advantage is resistance to yellowing upon prolonged exposure to sunlight.

The present invention has been described with respect to shade cloth, but it will be apparent

that the invention applies to other types of cellulose derivative coated fabrics and the term "window shade material" as used herein and in the appended claims is intended to include cellulose ester coated fabrics in general having properties similar to shade cloth, such as, e. g., sign cloth used in buses, trolley cars, etc., as illuminated signs.

It is apparent that many widely different embodiments of this invention may be made without departing from the spirit and scope thereof, and therefore, it is not intended to be limited except as indicated in the appended claims.

I claim:

15. A non-tendering window shade material comprising a fabric base having a film superposed thereon consisting essentially of cellulose nitrate, a plasticizer, and pigment, at least 20% of the said pigment comprising zinc oxide having a particle size greater than .4 micron and less than about 3.2 microns in any one direction.

20. A window shade material resistant to tendering and color change comprising a fabric coated on each side with a composition consisting essentially of cellulose nitrate, plasticizer, and zinc oxide, said zinc oxide having a particle size greater than .4 micron and less than about 3.2 microns in any one direction.

25. A window shade material resistant to tendering and color change upon prolonged exposure to sunlight comprising a cotton fabric base coated on each side with a composition comprising cellulose nitrate 40.6-53.8 parts, plasticizer 31.4-28.2 parts and pigment 18.0-28.0 parts, at least 20% of total pigment content consisting of zinc oxide having a particle size greater than .4 micron and less than about 3.2 microns in any one direction.

ROBERT L. LESTER.